# EUROPEAN PATENT SPECIFICATION

(11) **EP 1 613 185 B1**
(45) Date of publication and mention of the grant of the patent: **02.07.2008**
(21) Application number: 04727364.4
(22) Date of filing: 14.04.2004
(51) Int. Cl.: A43B 7/32, A43B 7/34, A43B 7/36, A41D 31/00, F41H 5/04, A43B 13/12

(54) **USE OF A PUNCTURE RESISTANT TEXTILE STRUCTURE FOR SHOE SOLES**
VERWENDUNG EINER DURCHLÖCHERUNGSSICHEREN TEXTILSTRUKTUR FÜR SCHUHSOHLEN
UTILISATION D'UNE STRUCTURE TEXTILE RESISTANTE A LA PERFORATION POUR DES SEMELLES DE CHAUSSURES

(30) Priority: 14.04.2003 IT PO20030005
(43) Date of publication of application: 11.01.2006
(73) Proprietor: Lenzi Egisto S.p.A., 59021 Vaiano (IT)
(72) Inventor: FENZI, Roberto, 59021 Vaiano (Prato) (IT)
(74) Representative: Bottero, Carlo
(86) International application number: PCT/IT2004/000208
(87) International publication number: WO 2004/089143

(56) References cited:
- WO-A-01/51263
- WO-A-01/68361
- US-A- 5 480 706
- US-A- 5 677 029
- US-A- 5 880 042

## Description

### Technical Field

This invention concerns the use of a textile structure in the field of footwear, particularly safety footwear, which is required to have a high level of resistance to penetration by sharp objects such as nails and the like, especially through the sole.

### Background Art

There are known systems of composite structures used for shoe soles in safety footwear designed to protect the feet from sharp or pointed objects. Some of these systems use metal plates which, however, add weight and reduce the flexibility of the shoe. The high thermal conductivity of the metal plate also makes the shoes uncomfortable to wear under conditions of high temperature. In addition; there are further problems when they are worn in places subject to the surveillance of metal detectors.

Document US 5480706 discloses a fire resistant multilayer complex ballistic resistant article comprising at least one first layer comprised a plurality of flammable fibers a first matrix and at least one second layer which is adjacent to said first layer which comprises a plurality of fire resistant fibers in a second matrix, wherein the second matrix comprises a fire retardant material and is different from the first matrix material.

Document WO 01/68361 shows a flexible article of manufacture especially suitable for use as a ballistic resistant body armor which comprises two or more layers, at least one of said layers being a fibrous layer, and at least one of said layers being a polymeric layer in contact with and bound to all or portion of said fibrous layer.

Document US 5677029 discloses a multilayered material for the protection of body parts from penetrating objects, comprising at least one energy-distributing layer and at least one energy-absorbing layer, as well as a protective insert for boots, a protective boot and a protective outer garment by using such a multilayered material.

Other systems make use of layers of fabrics made of aramidic fibers bonded together by a film of thermoplastic polymers (see, for example, patent US6368989). The difficulty with protective panels of this kind is that they are very expensive, due to the use of aramidic fibers only.

### Disclosure of Invention

The main object of this invention, therefore, is to provide a protective textile structure to be used in footwear, particularly shoe soles, which structure offers high resistance to piercing and penetration by sharp and pointed objects, while having limited thickness and weight, adequate flexibility and reduced cost.

A further object of this invention is to provide a perforation-resistant textile structure that is also antistatic and/or resistant to high temperatures.

These objects are achieved with the use of a perforation-resistant textile structure in conformity with enclosed claim1. Advantageous forms of implementation of the invention are defined in the dependent claims.

The advantages and technical characteristics of the invention will appear clear from the following detailed description of two non-limiting examples of its implementation.

### Brief Description of Drawings

In the drawings:
- Fig. 1 is a schematic illustration of a first textile structure in conformity with the invention;
- Fig. 2 shows the polyester fabric used in the structure of Fig. 1;
- Fig. 3 and 4 illustrate, respectively, the profile of the warp and weft of the fabric in Fig. 2;
- Fig. 5 is a schematic illustration of a second textile structure in conformity with the invention.

### Modes of Implementation of the Invention

With reference to Fig. 1 and 5, a textile structure 10,10' resistant to perforation in conformity with the invention basically consists of a number of layers 12,14,12',14' of woven fabrics bonded together by means of a thermoplastic film. In particular, the structure consists of one or more layers 12,12' of woven aramidic fibers and one or more layers of high tenacity non-aramidic fibers (for example, polyamide, polyester, polyolefin, liquid crystal fibers) woven into a fabric structure. Each separate layer of fabric has, preferably on the right side, a treated surface 16 coated with a polyurethane and/or acrylic resin reinforced with powders of hard, abrasive substances, preferably micronized ceramic materials in the form of silicates, e.g. of aluminum.

In the structure, the layers of aramidic fibers can be individually alternated with layers of fabric in non-aramidic fibers.

Two textile structures, as described more in detail hereafter, have been found to be particularly effective as well as practical to produce.

With reference to Figures 1 to 4, a first textile structure resistant to perforation consists of a multilayer structure 10 including a layer 12 of a woven fabric in aramidic fibers and, stacked on this layer 12, three layers 14 of a woven fabric in high tenacity polyester fiber. The layers are bonded together by means of a thermoplastic film. At least one side of each layer has been provided with a surface ceramic treatment 16.

Advantageously, the layers of fabric 12,14 are treated on the right side of the surface, the layer of aramidic fabric 12 and the adjacent layer 14 of polyester fabric with the treated surface 16 being in contact, the remaining layers of polyester fabric having the treated surface in contact with the untreated surface of the adjacent layer. In this way, both outer surfaces of the multilayer structure 10 are untreated. It is also advantageous to use the structure described above inside the soles of footwear with the layer in aramidic fibers on the tread side.

Thanks to the coating of ceramic material on the individual layers of fabric, a structure usable in conformity with this invention has high mechanical resistance to perforation by pointed metal objects and impedes their progress through the layers of fabric.

In addition, this structure is advantageously characterized by the fact of being composed in a proportion that does not exceed about 15 % by weight - of the total weight of the textile fibers used - of aramidic fibers, with the remaining part in high tenacity polyester fibers. This greatly reduces the production costs with respect to structures consisting entirely of aramidic fibers, maintaining it on the order of the production costs of structures consisting of metal plates, over which it has the advantage of being highly flexible.

In the practical implementation of a protective structure in conformity with the invention, it has been found to be particularly advantageous to select fabrics 12,14 forming the multilayer structure 10 described above in the following way.

Fabric in aramidic fibers:
- plain weave;
- warp yarns in aramidic fibers, specifically Kevlar® 730 dtex, density 19 ± 2% per cm;
- weft yarns in aramidic fibers, specifically Kevlar® 730 dtex, density 15 ± 2% per cm;
- ceramic surface layer applied by coating with 90 ÷ 120 gr/sq.mt. of a compound consisting of 50% polyurethane resin, 25% acrylic resin, and 25% aluminum silicate.

The fabric produced in this way has a finished weight of 340 ÷ 350 ± 5% gr/sq.mt. with a composition by weight of approximately 80% Kevlar ®, 10% polyurethane, 5% acrylic, 5% aluminum silicate.

Fabric in polyester fibers:
- compound weave (illustrated in Figures 2 to 4), made up of two simple weaves 3X3;
- warp yarns in high tenacity (H.T.) polyester fiber 1100 dtex, density 22 ± 2% per cm;
- weft yarns in high tenacity polyester fiber 1100 dtex, density 29 ± 2% per cm;
- ceramic surface layer applied by coating with 90 + 120 gr/sq.mt.

The fabric produced in this way has a finished weight of 690 + 720 ± 5% gr/sq.mt. with a composition by weight of approximately 86% polyester fibers, 7% polyurethane, 3.5% acrylic, 3.5% aluminum silicate.

The weaves used make it possible to produce fabrics with very tightly woven yarns, making their structure highly cohesive to provide by their very construction a good resistance to penetration, while maintaining a high degree of flexibility.

In particular, the compound weave used for the fabric in polyester fiber has been found to be particularly effective in the production of the multilayer structure 10.

The bonding between the layers of fabric is obtained by hot calandering with the insertion of a thermoplastic film (polyolefin and/or polyurethane and/or polyester) between the layers of the structure; processing the combination with heat causes the bonding by merger of the ceramic material both with the thermoplastic film and with the surface layer of the adjacent fabric layer so as to obtain a single unit with a total thickness of not more than 3 mm and limited weight.

Advantageously, using thermoplastic film made of polyester that is resistant to high temperatures, a structure can be obtained that is particularly suitable for footwear designed to be used in the presence of high heat sources.

The textile structure described above has a general composition of:
- aramidic fibers by weight in a percentage of approximately 12%.;
- high tenacity polyester fibers by weight in a percentage of approximately 73%.;
- surface treatment in ceramic by weight in a percentage of approximately 15%.
- total weight 2435 ÷ 2555 ± 5% gr/sq.mt..

Tests carried out on the structure have proven its effective resistance to a force of at least 1100N exerted by a nail, as foreseen by standards pr EN ISO 20344, EN 344/92 and EN 12568/98.

By inserting electrically conductive wires in the fabric of the aramidic fibers and in the fabrics in non-aramidic fibers composing the multilayer structure, an antistatic structure is obtained which can be used in footwear for which this feature is required.

In particular, it is advantageous to produce the fabric in aramidic fibers with:
- the warp yarns consisting, every 74 threads, of a first yarn repeated 73 times in Kevlar® 730 dtex and a second yarn repeated once in high tenacity polyamide 180 dtex in two ply twisted with a filament in stainless steel measuring 60 micron in diameter (a composition thus consisting of 82% polyamide and 18% stainless steel);.
- the weft yarns consisting, every 56 wefts, of a first weft repeated 55 times in Kevlar® 730 dtex 730 and a second weft repeated once in polyamide and steel as described above.

The fabric in polyester fiber is in turn preferably produced with:
- 23 ± 2% warp threads per cm consisting, every 24 threads, of a first yarn repeated 23 times in polyester H.T. 1100 dtex and a second thread repeated once in polyester H.T. 1100 dtex plus a twisted filament of carbon (or steel) 24 dtex (final composition 95 % polyester 5% carbon);
- 25.5 ± 2% weft yarns per cm consisting, every 30 wefts, of a first weft repeated 28 times in polyester H.T. 1100 dtex and a second weft repeated twice in polyester H.T. and carbon as described above.

A second example of a textile structure resistant to perforation usable in conformity with the invention is schematically illustrated in Fig. 5.

In this case the structure 10' includes two bonded multilayers 120,140, consisting of a first set of three stacked layers of a woven fabric 12' in aramidic fibers provided with a surface ceramic treatment 16 and a second set of three stacked layers of a woven fabric 14' in high tenacity polyamide provided with a surface ceramic treatment. Advantageously, at least two adjacent layers 12' of fabric in aramidic fibers or two adjacent layers of fabric 14' in polyamide fibers or the two adjacent layers of the multilayer structures 120,140 have the treated surfaces 16 in contact with each other so that both the outer surfaces (top and bottom) of the structure 10' are not treated.

In practical implementation, it has been found to be particularly advantageous to select the fabrics forming the multilayer structures 120,140 described above in the following way.

Fabric in aramidic fibers: as in the first example described above.

Fabric in polyamide fibers:
- weft rep weave;
- warp yarns in polyamide 6:6 high tenacity fiber, 200 dtex, taslanized and density 62 per cm;
- weft yarns in high tenacity nylon 6:6, 636 dtex, taslanized and density 16.5 per cm;
- surface layer of ceramic applied by coating of 60 gr/sq.mt. of the same compound described above.

The fabric produced in this way has a finished weight of about 300 gr/sq.mt. with a composition by weight of 80% of polyamide fibers, 10% polyurethane, 5% acrylic, 5% aluminum silicate.

A structure composed of three layers of fabric in aramidic fibers and three layers of fabric in high tenacity polyamide as described above, has a general composition of
- aramidic fibers by weight in a percentage of approximately 38%.;
- high tenacity polyamide fibers by weight in a percentage of approximately 34%.;
- ceramic surface treatment by weight in a percentage of approximately 18%.;
- total weight approximately 2200 gr/sq.mt.
the thickness is under 3 mm (after bonding of the layers by hot calandering and insertion of thermoplastic film).

A textile structure capable of resisting penetration, as described in the above examples, is also thermally insulating and can be used, in the traditional way, as a protective insert into soles which are applied to footwear by means of sewing or gluing.

According to the invention, this structure is used in the production of footwear the sole of which is directly made on the upper by injection molding. In Strobel type footwear, this structure constitutes the insole, which is first sewn onto the upper after which the sole is injected. It has been ascertained, in fact, that the effective resistance to perforation and penetration of a nail, according to the terms of standard EN 344/92, does not prevent sewing the structure onto the upper, using needles of an appropriate type.

The invention thus conceived is susceptible to numerous alterations and variations within the scope of the appended claims.

## Claims

1. Use of a textile structure resistant to perforation in the production of footwear in which the sole is directly produced on the upper by injection molding, as an insole that is first sewn to the upper of the footwear, wherein said textile structure (10) comprises one or more layers (12, 12') of woven aramidic fibers and one or more layers (14, 14') of high tenacity woven non-aramidic fibers, said layers being bonded together by means of thermoplastic film, each individual woven layer being treated by coating with a polyurethane and/or acrylic resin enriched with powders of hard and abrasive materials.

2. Use of a textile structure according to claim 1 wherein said hard and abrasive materials are ceramic materials, preferably micronized and in the form of silicates.

3. Use of a textile structure according to claim 2 wherein said micronized ceramic materials are aluminum silicates.

4. Use of a textile structure according to one of the claims from 1 to 3, wherein a multilayer structure includes a first layer of a woven fabric made of aramidic fibers and, stacked on the first layer, three layers of a woven fabric made of high tenacity polyester fibers, the layers being bonded together by means of thermoplastic film and at least one side of each layer being provided with a surface ceramic treatment.

5. Use of a textile structure according to claim 4, wherein the layer of aramidic fabric and the adjacent layer of polyester fabric have the treated surfaces placed in contact, the remaining layers of polyester fabric having the treated surface in contact with the untreated surface of the adjacent layer.

6. Use of a textile structure according to claim 4, wherein not more than 15-20% by weight of the total by weight of the textile fibers used consists of aramidic fibers.

7. Use of a textile structure according to claim 5, wherein:
- the fabric in aramidic fibers is a plain weave fabric having warp yarns in aramidic fibers, specifically Kevlar^{®} 730 dtex, 19 yarns per cm, and weft yarns in aramidic fiber, specifically Kevlar^{®} 730 dtex, 15 yarns per cm, coated on the right side with 90-120 gr/sq. mt. of a compound consisting of 50% polyurethane resin, 25% acrylic resin, 25% aluminum silicate;
- the fabric in polyester fiber is a compound weave fabric, made up of two simple weaves 3X3, with the warp and weft yarns in polyester H.T. 1100 dtex, 22 per cm and 29 per cm respectively, and is coated on one side with said compound.

8. Use of a textile structure according to one of the claims from 4 to 7, wherein electrically conductive wires are inserted in the fabric in aramidic fibers and in the fabric in high tenacity non-aramidic fibers composing said multilayer structure.

9. Use of a textile structure according to one of the claims from 1 to 3, wherein the layers of fabric in aramidic fibers are individually alternated with those in high tenacity non- aramidic fibers.

10. Use of a textile structure according to one of the claims from 1 to 3, wherein two multilayer structures of fabric are bonded, one consisting of three stacked layers of a woven fabric in aramidic fibers treated on the surface with a ceramic coating and the second consisting of three layers of a woven fabric in high tenacity polyamide fibers treated on the surface with a ceramic coating.

11. Use of a textile structure according to claim 10, wherein two adjacent layers of fabric in aramidic fibers or two adjacent layers of fabric in polyamide fibers, or the two adjacent layers of the multilayer structures have the treated surfaces in contact, the external surfaces on the top and bottom of the structure being not treated.

12. Use of a textile structure according to claim 10, wherein not more than 50-60% by weight of the total weight of the textile fibers used consists of aramidic fibers.

13. Use of a textile structure according to claim 10, wherein:
- the fabric in aramidic fibers is a plain weave fabric, having the warp yarns in aramidic fiber, specifically Kevlar^{®} 730 dtex, 19 yarns per cm and weft yarns in aramidic fiber, specifically Kevlar^{®} 730 dtex, 15 yarns per cm, coated on the right side with 90-120 gr/sq.mt. of a compound consisting of 50% polyurethane resin, 25% acrylic resin,25% aluminum silicate;
- the fabric in polyamide fibers is a weft rep weave fabric, having warp yarns in high tenacity polyamide 6:6 fiber, 200 dtex, taslanized, 62 per cm, and weft yarns in high tenacity Nylon 6:6, 636 dtex, taslanized, 16.5 per cm., coated on the right side with 60gr/sq. mt. of said compound.

14. Use: of a textile structure according to claim 1, wherein the aforementioned thermoplastic films are made of polyester which resists to high temperatures.

## Patentansprüche

1. Verwendung einer bruchfesten Textilstruktur bei der Herstellung von Schuhen, bei den die Sohle unmittelbar auf dem Obermaterial durch Spritzgießen als eine Einlegesohle hergestellt wird, die erst mit dem O-bermaterial der Schuhe zusammengenäht wird, worin die benannte Textilstruktur (10) eine oder mehrere Schichten (12, 12') aus gewebten Aramidfasern und eine oder mehrere Schichten (14, 14') aus hochfesten gewebten Nichtaramidfasern umfasst, wobei die benannte Schichten durch thermosplastischesfilm zusammenverbunden sind, wobei jede einzelne gewebte Schicht durch Beschichtung mit einem Polyurethan- und/oder Acrylharz, das mit Pulvern aus harten und Schleifmaterialien angereichert sind, behandelt ist.

2. Verwendung einer Textilstruktur nach Anspruch 1, worin die benannten harten und Schleifmaterialien Keramikmaterialien, bevorzugt micronisierten Materialien in Form von Silikaten, sind.

3. Verwendung einer Textilstruktur nach Anspruch 2, worin die benannten micronisierten Keramikmaterialien Aluminiumsilikaten sind.

4. Verwendung einer Textilstruktur nach einem der Ansprüche 1 bis 3, worin eine multischichtige Struktur eine erste Schicht aus einem Gewebe aus Aramidfasern und drei auf die erste Schicht gestapelte Schichten aus einem Gewebe aus hochfesten Polyesterfasern umfasst, wobei die Schichten durch thermoplastischefilm zusammenverbunden sind und mindestens eine Seite von jeder Schicht mit einer keramischen Oberflächenbehandlung vorgesehen ist.

5. Verwendung einer Textilstruktur nach Anspruch 4, worin die Schicht aus Aramidgewebe und die anliegende Schicht aus Polyestergewebe die behandelten Oberflächen in gegenseitiger Berührung aufweisen, wobei die verbleibenden Schichten aus Polyestergewebe die behandelte Oberfläche in Berührung mit der nichtbehandelten Oberfläche der anliegenden Schicht aufweisen.

6. Verwendung einer Textilstruktur nach Anspruch 4, worin nicht mehr als 15-20 Gew.-% des Gesamtgewichtes der verwendeten Textilfasern aus Aramidfasern besteht.

7. Verwendung einer Textilstruktur nach Anspruch 5, worin
- das Gewebe aus Aramidfasern ein Taftbindungsgewebe ist, mit den Kettenfäden aus Aramidfasern, insbesondere Kevlar^{®} 730 dtex, 19 Fäden pro cm, und den Schussfäden aus Aramidfasern, insbesondere Kevlar^{®} 730 dtex, 15 Fäden pro cm, mit einer Beschichtung auf der rechten Seiten mit 90-120 g/m² einer Verbundwerkstoff aus 50% Polyurethanharz, 25% Acrylharz, 25% Aluminiumsilikat;
- das Gewebe aus Polyesterfasern ein Verbundbindungsgewebe ist, bestehend aus zwei einfachen 3X3 Bindungen, mit den Kettenfäden und den Schussfäden aus hochfestem Polyester, 1100 dtex, 22 pro cm bzw. 29 pro cm, mit einer Beschichtung auf einer Seite mit der benannten Verbindung.

8. Verwendung einer Textilstruktur nach einem der Ansprüche 4 bis 7, worin elektrisch leitfähige Drahte in das Gewebe aus Aramidfasern und in das Gewebe aus hochfesten Nichtaramidfasern, die die benannte multischichtige Struktur bilden, eingeführt werden.

9. Verwendung einer Textilstruktur nach einem der Ansprüche 1 bis 3, worin die Gewebeschichten aus Aramidfasern einzeln mit den Gewebeschichten aus hochfesten Nichtaramidfasern alterniert werden.

10. Verwendung einer Textilstruktur nach einem der Ansprüche 1 bis 3, worin zwei multischichtige Gewebestrukturen verbunden werden, die eine bestehend aus drei gestapelten Schichten aus einem Gewebe aus Aramidfasern, das auf der Oberfläche mit einer keramischen Beschichtung behandelt ist, und die zweite bestehend aus drei Schichten aus einem Gewebe aus hochfesten Polyamidfasern, das auf der Oberfläche mit einer keramischen Beschichtung behandelt ist.

11. Verwendung einer Textilstruktur nach Anspruch 10, worin zwei anliegende Gewebeschichten aus Aramidfasern oder zwei anliegende Gewebeschichten aus Polyamidfasern, oder die beiden anliegenden Schichten der multischichtigen Strukturen die behandelten Oberflächen in gegenseitiger Berührung aufweisen, wobei die Außenoberflächen oben und unten der Struktur nicht behandelt sind.

12. Verwendung einer Textilstruktur nach Anspruch 10, worin nicht mehr als 50-60 Gew.-% des Gesamtgewichtes der verwendeten Textilfasern aus Aramidfasern besteht.

13. Verwendung einer Textilstruktur nach Anspruch 10, worin:
- das Gewebe aus Aramidfasern ein Taftbindungsgewebe ist, mit den Kettenfäden aus Aramidfasern, insbesondere Kevlar^{®} 730 dtex, 19 Fäden pro cm, und den Schussfäden aus Aramidfasern, insbesondere Kevlar^{®} 730 dtex, 15 Fäden pro cm, mit einer Beschichtung auf der rechten Seiten mit 90-120 g/m² einer Verbundwerkstoff aus 50% Polyurethanharz, 25% Acrylharz, 25% Aluminiumsilikat;
- das Gewebe aus Polyamidfasern ein Schussripsbindungsgewebe ist, mit den Kettenfäden aus hochfesten 6;6-Polyamidfasern, 200 dtex, taslanisiert, 62 pro cm, und den Schussfäden aus hochfestem 6:6-Nylon, 636 dtex, taslanisiert, 16,5 pro cm, mit einer Beschichtung auf der rechten Seite mit 60 g/m² der benannten Verbindung.

14. Verwendung einer Textilstruktur nach Anspruch 1, worin die oben genannten thermoplastischefilme aus hochtemperaturfestem Polyester bestehen.

## Revendications

1. Utilisation d'une structure textile résistante à la perforation dans la production de chaussures dans lesquelles la semelle est réalisée directement sur la tige par moulage par injection, comme semelle intérieure étant tout d'abord cousue sur la tige de la chaussure, où ladite structure textile (10) comprend une ou plusieurs couches (12, 12') de fibres aramide tissées et une ou plusieurs couches (14, 14') de fibres non-aramide tissées à haute ténacité, lesdites couches étant liées l'une à l'autre au moyen de film thermoplastique, chaque couche tissée individuelle étant traitée par revêtement avec une résine polyuréthane e/ou acrylique enrichie avec des matériaux durs et abrasifs en poudre.

2. Utilisation d'une structure textile selon la revendication 1, où lesdits matériaux durs et abrasifs sont matériaux céramiques, de préférence micronisés et en forme de silicates.

3. Utilisation d'une structure textile selon la revendication 2, où lesdits matériaux céramiques micronisés sont silicates d'aluminium.

4. Utilisation d'une structure textile selon une des revendications 1 à 3, où une structure multi-couche comporte une première couche d'un tissu tissu en fibres aramides et, empilées sur la première couche, trois couches d'un tissu tissu en fibres polyester à haute ténacité, les couches étant liées l'une à l'autre au moyen de film thermoplastique et au moins un côté de chaque couche étant muni d'un traitement céramique de surface.

5. Utilisation d'une structure textile selon la revendication 4, où la couche de tissu aramide et la couche adjacente de tissu polyester ont les surfaces traitées en contact entre elles, les couches restantes de tissu polyester ayant la surface traitée en contact avec la surface non-traitée de la couche adjacente.

6. Utilisation d'une structure textile selon la revendication 4, où non plus de 15-20% en poids du total en poids des fibres textiles utilisées se compose de fibres aramide.

7. Utilisation d'une structure textile selon la revendication 5, où:
- le tissu en fibres aramide est un tissu à armure toile ayant les fils de chaîne en fibres aramide, notamment Kevlar® 730 dtex, 19 fils par cm, et les fils de trame en fibres aramide, notamment Kevlar® 730 dtex, 15 fils par cm, revêtu sur le côté droit avec 90-120 g/m² d'un composition consistant de 50% de résine polyuréthane, 25% de résine acrylique, 25% de silicate d'aluminium;
- le tissu en fibres polyester est un tissu à armure composite, consistant de deux armures simples 3X3, avec les fils de chaîne et de trame en polyester à haute ténacité, 1100 dtex, respectivement 22 par cm et 29 par cm, et revêtu sur un côté avec ledit composé.

8. Utilisation d'une structure textile selon une des revendications 4 à 7, où des fils électriquement conducteurs sont insérés dans le tissu en fibres aramide et dans le tissu en fibres non-aramide à haute ténacité composant ladite structure multi-couche.

9. Utilisation d'une structure textile selon une des revendications 1 à 3, où les couches de tissu en fibres aramide sont alternées chacune avec celles en fibres non-aramide à haute ténacité.

10. Utilisation d'une structure textile selon une des revendications 1 à 3, où deux structures multi-couche de tissu sont liées l'une à l'autre, l'une consistant de trois couches empilées d'un tissu en fibres aramide traité en surface avec un revêtement céramique, et la deuxième consistant de trois couches d'un tissu en fibres polyamide à haute ténacité traité en surface avec un revêtement céramique.

11. Utilisation d'une structure textile selon la revendication 10, où deux couches adjacentes de tissu en fibres aramide ou deux couches adjacentes de tissu en fibres polyamide, ou les deux couches adjacentes des structures multi-couche ont les surfaces traitées en contact, les surfaces extérieures sur le sommet et au fond de la structure étant non-traitées.

12. Utilisation d'une structure textile selon la revendication 10, où non plus de 50-60% en poids du total en poids des fibres textiles utilisées se compose de fibres aramide.

13. Utilisation d'une structure textile selon la revendication 10, où;
- le tissu en fibres aramide est un tissu à armure toile, ayant les fils de chaîne en fibres aramide, notamment Kevlar® 730 dtex, 19 fils par cm, et les fils de trame en fibres aramide, notamment Kevlar® 730 dtex, 15 fils par cm, revêtu sur le côté droit avec 90-120 g/m² d'un composition consistant de 50% de résine polyuréthane, 25% de résine acrylique, 25% de silicate d'aluminium;
- le tissu en fibres polyamide est un tissu à armure reps de trame, avec les fils de chaîne en fibres polyamide 6:6 à haute ténacité, 200 dtex, taslanisé, 62 par cm, et les fils de trame en Nylon 6:6 à haute ténacité, 636 dtex, taslanisé, 16,5 par cm, et revêtu sur le côté droit avec 60 g/m² dudit composé.

14. Utilisation d'une structure textile selon la revendication 1, où les sus-mentionnés films thermoplastique sont en polyester résistant aux hautes températures.
